

Oct. 22, 1974

S. RUSSELL ET AL

3,843,497

ELECTROLYTIC PRODUCTION OF BORON

Original Filed June 17, 1969

2 Sheets-Sheet 1

FIG. 1



Oct. 22, 1974

S. RUSSELL ET AL

3,843,497

ELECTROLYTIC PRODUCTION OF BORON

Original Filed June 17, 1969

2 Sheets-Sheet 2

FIG. 2.



FIG. 3



**1**

3,843,497

**ELECTROLYTIC PRODUCTION OF BORON**

Sid Russell, Suffield, Frederick A. Young, Simsbury, and Jordan D. Kellner, West Suffield, Conn., assignors to United Aircraft Corporation, East Hartford, Conn. Continuation of abandoned application Ser. No. 833,913, June 17, 1969. This application Mar. 13, 1972, Ser. No. 234,306

Int. Cl. C23b 5/00; C22d 3/00

U.S. Cl. 204—64 R

**8 Claims****ABSTRACT OF THE DISCLOSURE**

A process for producing substantially pure coherent boron on a cathode by electrodeposition from a fused salt bath comprising an alkali or alkaline earth metal fluoride or mixture of fluorides by establishing in the bath a fluoborate ion concentration not exceeding about 20 percent by weight and heating the bath to a temperature of about 1000°—1400° F. in a non-contaminating atmosphere and establishing a current density at the cathode not exceeding about 400 milliamperes per square centimeter.

This is a continuation of application Ser. No. 833,913, filed June 17, 1969, now abandoned.

**BACKGROUND OF THE INVENTION**

This invention relates to electrochemical processes and more particularly relates to an electrolytic process for depositing substantially pure coherent boron coatings from a fused haloborate bath.

It is known that coatings of essentially pure boron up to several mils in thickness may be produced by pyrolytic techniques wherein the boron is deposited on a resistively heated wire which is drawn through a gaseous reactant stream. Early investigations quickly revealed the utility of these fibers for a variety of applications including the production of fiber-reinforced articles having improved physical properties.

Although the technique of gas phase deposition of boron results in high density continuous coatings, there remain several inherent limitations therein. The process, in requiring the reaction of a boron containing gas with hydrogen gas, engenders problems associated with dual gas flow metering and mixing, flow pattern control, and uniform temperature control. Further, the size and shape of substrates which can be coated are severely limited, and only very few substrate materials are compatible with the coating process due to the high temperatures involved.

Although it is known in the prior art to obtain elemental boron by electrolysis from molten salts, it has not been possible to obtain the boron as a pure coating of substantial thickness. Primarily, the prior electrolytic techniques have produced coatings of granular boron containing a high percentage of occluded electrolyte salts. In order to obtain substantially pure boron, secondary processing to leach out the salts has been necessary. Unfortunately, such processing destroys the coating and results in loose boron powder.

Thus, the great desirability of electrolytically producing a salt-free boron electroplate is well recognized but thus far has not been achieved by prior processes.

**SUMMARY OF INVENTION**

In accordance with this invention, means have been formulated to provide by electrolytic deposition a substantially pure coherent electroplate of boron of essentially unlimited thickness upon a variety of substrates including those not readily amenable to the gas phase process. The present invention contemplates the precise control of critical processing variables such as temperature, current density and electrolyte composition in a fused salt

**2**

electrolyte comprised of an alkali or alkaline earth metal fluoride or mixture of fluorides and containing fluoborate ions. In a preferred embodiment, the invention contemplates a pretreatment of the electrolyte, prior to electrolysis, to reduce the concentration of contaminating agents to a level below that which has been found to interfere with the deposition process. In brief, the present invention permits the production of coherent boron coatings of from 85 to 100% purity by the establishment of a fluoborate ion concentration up to 20% by weight of the bath, a current density up to 400 m./cm.<sup>2</sup> and a temperature between 1000° and 1400° F.

**BRIEF DESCRIPTION OF THE DRAWINGS**

FIG. 1 is a view of an electrolytic cell, taken in elevation and partially in cross section, which is suitable for use in the practice of the present invention;

FIG. 2 is a graph illustrating the relation between current density and BF<sub>3</sub> concentration; and

FIG. 3 is a graph illustrating the relation between current density and temperature.

**DESCRIPTION OF THE PREFERRED EMBODIMENTS**

Referring first to FIG. 1, the electrolytic cell is designated generally by the numeral 10 and includes a graphite or carbon crucible 12 placed inside a heat resistant, metal shell or pot 14 made of nickel or other suitable metal. The outer pot 14 is fitted with a covering lid 16 having an air-lock 17 so that the melt can be kept under an inert atmosphere during electrolysis as well as during a change of cathodes. The cell is externally heatable by an electric resistance furnace 18 surrounding the lower portion of the cell. The crucible 12 is filled or partially filled with an electrolyte 20 in which are suspended an anode 22 and a cathode 24.

The fused salt electrolyte 20, sometimes referred to hereinafter as a fused salt bath, comprises preferably the fluorides and fluoborates of the alkali and alkaline earth metals, such as lithium, sodium, potassium, barium, calcium, strontium and others which have a reduction potential more negative than that required for boron deposition, with the bath containing up to 20 weight percent fluoborate ions. In general, the temperature of the fused salt bath is maintained within the range of from approximately 1000° to 1400° F., the exact temperature required being dependent upon the concentration of fluoborate in the electrolyte, the current density at which the boron is being plated, and the physical configuration of the cell.

In a preferred embodiment of the process for plating pure boron coatings, a mixture of lithium fluoride and potassium fluoride is used as an electrolyte base. A mixture comprising 40 to 60 mol percent lithium fluoride and 60 to 40 mol percent potassium fluoride is satisfactory.

It is to be noted that electrolyte contaminants such as heavy metal ions must be kept out of the electrolyte. By utilizing the cell configuration shown in FIG. 1, the electrolyte contacts carbon structural materials only and this objective is achieved.

In order to reduce the starting concentration of dissolved gases, the base halide salts are preferably subjected, before the addition of boron in any form, to a vacuum at a temperature just below their melting point for a period sufficient to achieve an equilibrium pressure of 10<sup>-4</sup> mm. Hg. After the foregoing pretreatment, a fluoborate forming compound such as BF<sub>3</sub> gas, itself purified of oxygen containing gases, is added to the base halide salts in appropriate amounts to produce the desired concentration of fluoborate ions. A concentration up to 20 percent by weight of fluoborate ion content in the electrolyte is considered satisfactory, although a content between 2 and 10 percent

by weight is preferred. It will be appreciated by those skilled in the art that the heat-vacuum conditioning treatment of the base halide salts must be carried out prior to the introduction of the  $\text{BF}_3$  and consequent formation of fluoborate in the melt since, with fluoborate present, the decontamination of the electrolyte by vacuum treatment cannot be effectively accomplished due to the fact that the outgassing of  $\text{BF}_3$  from the electrolyte restricts the level of pressure to which the system can be evacuated.

In an alternative pretreatment technique, the electrolyte can be purified subsequent to the formation of fluoborate. In this procedure, the base halide salts are melted and a fluoborate forming compound such as  $\text{BF}_3$  gas or  $\text{KBF}_4$  powder is added. The electrolyte is then conditioned by the addition of a reducing element such as elemental boron. The boron reacts with dissolved gases and vapors such as water, oxygen and carbon dioxide and also with oxianionic contaminants, such as carbonate and hydroxide to reduce their concentration to below interfering levels. It is to be noted that heavy metals in solution also are reduced out of solution by the elemental boron.

In the practice of the invention, a carbon crucible 4 inches in diameter and 10 inches in depth was used. Reagent grade anhydrous salts,  $\text{KF}$  (1385 grams) and  $\text{LiF}$  (615 grams), were weighed quickly in air to prevent excessive moisture pickup and then placed in a vacuum oven at  $180^\circ \text{ C}$ . for several days. The hot, partially dried salts were then transferred to a similarly baked out carbon crucible and installed quickly within the electrolytic cell, which was then evacuated to  $10^{-4} \text{ mm. Hg}$  for at least 24 hours at  $450^\circ \text{ C}$ . In general, subjecting the fluorides to a temperature of from  $110^\circ$  to  $480^\circ \text{ C}$ . at a pressure from  $10^{-2}$  to  $10^{-6} \text{ mm. Hg}$  for up to 200 hours is satisfactory. Argon gas, which was passed through a magnesium perchlorate drier and a bed of hot copper turnings to remove oxygen, was then introduced over the salts and the temperature was raised to  $700^\circ \text{ C}$ . to melt the salts. Tests showed that after the aforesaid hard vacuum-high temperature treatment, the residual dissolved moisture and gases, as determined by direct measurements of water, carbon dioxide, and carbon monoxide in the argon purge gas, was extremely small. Carbon dioxide and carbon monoxide have proved to be particularly effective indicators of contamination level since water and oxygen, which are the most important contaminants, react with the carbon crucible to produce these gases. It has been determined that a satisfactorily purified melt exhibits less than 10 p.p.m./v. each of carbon monoxide and carbon dioxide in the purge gas at a flow rate of  $30 \text{ cm}^3/\text{min}$ .

The residual contamination level was also determined by voltammetry. It was found that the degree of residual oxianion contamination could be determined from the observed current when an anodic potential sweep (20 mv./min.) was made on a carbon electrode dipping into the conditioned melt. A current maximum was consistently observed when the potential reached about 1.5 volts more positive than a second carbon "quasi reference" electrode. The height of the current maximum could be related to the contamination level. Assignment of the current to oxianion discharge was possible from the observed elution of carbon dioxide and carbon monoxide from the working carbon electrode as measured in the argon purge gas. In a properly conditioned melt, that is, one containing contaminants at a non-interfering level, a maximum current of about 0.5 ma./ $\text{cm}^2$  was observed, again with less than 10 p.p.m./v. each of carbon dioxide and carbon monoxide in the effluent purge gas at a flow rate of  $30 \text{ cm}^3/\text{min}$ . Although a current maximum of 0.5 ma./ $\text{cm}^2$  or lower is preferred, satisfactory depositions have been made with current maximums up to 10 ma./ $\text{cm}^2$ .

When it was ascertained that the melt was sufficiently purified, commercially available  $\text{BF}_3$  gas was bubbled into the melt through a hollow carbon tube until the selected concentration of fluoborate ions was produced. The gas

was processed before entering the cell by passing it over steel wool heated to  $450^\circ \text{ F}$ . to remove air, sulfur dioxide, and other oxygen containing gases which are generally present in the commercial supplies, and then passed through a particulate filter to take out the boric oxide "smoke" formed in that process. Almost all of the  $\text{BF}_3$  added was absorbed by the melt, and therefore the fluoborate produced could be closely determined by the volume of gas introduced. However, confirmation of the precise fluoborate concentration was accomplished electrochemically by chronopotentiometry and by chemical analysis.

In an alternative technique, a less rigorous melt purification procedure is used and the  $\text{BF}_3$  makeup gas and the argon sweep gas need not be purified as described above. During experimentation, it was discovered that the concentration of dissolved contaminants can still be substantially controlled by treating the electrolyte containing the fluoborate with elemental boron. The boron additive reacts with interfering contaminants in the melt to reduce their concentration, although the exact action of the elemental boron is incompletely understood at this time. When boron is first added, evolution of a gas, suspected to be hydrogen, is generally observed. This ceases after a short period of time. The boron addition is then characterized by a decrease in the concentration of fluoborate in the electrolyte with an increase in the concentration of boron present as soluble ionic species other than fluoborate. Boron chips subsequently retrieved from the electrolyte, at times, show that heavy metals such as iron also are being reduced on their surfaces. When the electrolyte becomes passive to the further addition of elemental boron, the treatment is considered complete. It is presently believed that the elemental boron combines with both the fluoborate and dissolved contaminants to produce less interfering ionic boron oxifluoride species. It is desirable to use fine boron chips in the treatment, since the reaction with the electrolyte produces a coating on the boron surface which deactivates it, leading to long reaction time and material waste. The appropriate action of elemental boron is not accomplished under electrolysis if the boron is being used as an anode.

In the practice of boron plating, although graphite anodes were found satisfactory, the working anode preferred was a boron-filled carbon tube. The carbon tube used was one inch in diameter and stoppered at one end with a carbon plug and at the other end with a carbon plug and support rod. The tube used had approximately 80 holes,  $\frac{1}{32}$  inch in diameter, to permit the boron chips inside to be in contact with the electrolyte. The anodes were preferably assembled and baked out in an oven for several hours before use in order to remove absorbed oxygen and water. Since the amount of boron originally present in the anode was known, periodic checks on the amount of current passed were made as a means for determining the amount of boron remaining.

The cathodes most frequently used were generally pure copper strips  $\frac{1}{4}$  inch wide by  $2\frac{1}{2}$  inches long. Other materials, including carbon and molybendum, and other shapes were also coated. In general, any metal and alloy inert to the fused bath salts and suitable for use as a cathode may be boron plated. The copper strips were suspended from above using copper rods and were anodically cleaned in an alkaline cyanide bath, followed by rinses in water and dilute  $\text{HC1}$ , and finally dried with acetone. At times, as an alternative to the electrolytic cleaning, the copper cathodes were cleaned in dilute  $\text{HNO}_3$ .

During the plating operation, a constant slow sweep of purified inert gas, such as argon, was maintained over the electrolyte at a pressure slightly above atmospheric. The argon sweep is advantageous in that it prevents the inflow of atmospheric air and also facilitates periodic analyses of the effluent gas mixture from the cell. Over a period of time, however, there is a cumulative loss of  $\text{BF}_3$  gas from the system wherein the  $\text{BF}_3$  gas must be replenished.

Under varied combinations of operating parameters, boron coatings were obtained with five generally distinctive surface finishes. As shown in FIGS. 2 and 3, the coatings were produced under the operating conditions defined by the areas LMNO and WXYZ. All of the coatings were coherent, that is, they were continuous, homogeneous and in one piece. For convenience, the surface finishes have been classified as (A) a "mirror" finish, (B) a "steel" gray finish, (C) a "matte" finish, (D) a "velvet" finish, and (E) a "sooty" finish. The appearance of these coatings was characteristic of the geometry of the surface since the bulk of the coating appeared similar. The "mirror" finish coatings have very smooth flat surfaces while the "steel" gray finish coatings are characterized by scattered nodules which break up the reflection from the surface. The "matte" coatings have completely nodular surfaces. The "velvet" surface is covered with some microscopic granules, some of which can be rubbed off. The "sooty" coatings have a more powdery surface and a more appreciable amount of boron can be rubbed off. The coating bulk, in all cases, when broken showed the typical conchoidal fractures of amorphous boron.

Some of the coatings were examined by X-ray diffraction and showed the halo pattern typical of amorphous boron as is found for the pyrolytically deposited material.

Chemical analysis of the various coating types have shown variations in coating purity from 85% boron to substantially 100% boron with the purity showing a general correlation with the surface finishes which were obtained. The "mirror" finish coatings generally exhibit the lowest purities, while essentially pure coatings are obtained when surfaces appear "velvet" or "sooty." The lower purity of "mirror" finish coatings may be due to the formation of small microcracks and subsequent salt inclusion in openings, rather than to some intrinsic coating property. The coating type which presently promises wide utility is that which ranges between "velvet" and "matte" because it combines high purity with good surface characteristics.

The plated coatings were normally one or two mils thick, although thicknesses up to 23 mils were prepared on occasion. Some preliminary physical properties were determined for the coatings. Values for elastic modulus in flexure range between  $60 \times 10^6$  and  $70 \times 10^6$  p.s.i., and a Vickers hardness of approximately 3000 HV were measured. It will be appreciated that the later measurement is similar to the literature value for boron which is 2800 HV.

Further to the above properties, it was determined that the coatings produced by the present process were tightly adherent to the cathode. The boron plate formed an excellent bond to the copper, and coatings produced directly on carbon and molybdenum were also found to be highly adherent.

As indicated, the operating conditions for obtaining the various coatings are shown in FIGS. 2 and 3. From these graphs, it can be seen that, in general, by increasing the concentration of  $BF_3$  in the electrolyte, the same type coating is achieved at increasing current densities. By the same token, an increase in temperature has the effect of permitting the achievement of the same type coating at a higher current density. For example, at temperatures between  $1080^\circ$  and  $1350^\circ$  F., current densities of 15 ma./cm.<sup>2</sup> to 100 ma./cm.<sup>2</sup>, depending on the concentration of  $BF_4^-$  in the electrolyte, are necessary to produce smooth metallic coherent coatings of boron. Concentrations of about 1-3 weight percent  $BF_4^-$ , produce smooth coatings in the current density range of 15-50 ma./cm.<sup>2</sup> at temperatures above  $1200^\circ$  F. At concentrations of 3-7 weight percent  $BF_4^-$ , smooth coatings are obtained up to 100 ma./cm.<sup>2</sup> current density and down to  $1100^\circ$  F. temperature. With appropriate control over electrolyte  $BF_4^-$  concentration, temperature, and cathode operating current density, it is possible to select

and produce the desired type boron coating over a wide range of plating conditions.

While the present invention has been described with reference to the application of boron coatings directly to a material to be coated, it is appreciated that the described coating technique admits of wider application. It is recognized for example that the boron coating need not be direct and that copper, for example, may be used as a tie coat to promote bonding to other metal substrates. This technique has, for example, actually been used successfully to effect bonding to titanium and steel. It is also recognized that the process may be used in the production of such products as two dimensionally isotropic composite structures, which may be built up by plating successive coatings of boron and another material on each other. Such a composite was actually made using alternate coatings of boron and copper. Additionally, composite structures have been made using epoxy adhesive between successive sheets of boron coated copper foil.

For the sake of clarity, the foregoing description has been made with reference to particular materials, embodiments and operating parameters. It will be understood that these examples are illustrative only and that alternative materials, arrangements and operating conditions will be evident to those skilled in the art. Accordingly, the true scope of the invention will be measured, not by the illustrative material but rather, in the spirit of the invention, by the appended claims.

What is claimed is:

1. A process for producing substantially pure coherent boron on a cathode by electrodeposition from a fused salt bath consisting essentially of an alkali or alkaline earth metal fluoride or mixture of fluoride comprising: purifying the alkali or alkaline earth metal fluoride or mixture of fluorides until the residual oxianion contamination level therein is no greater than that amount which will produce a current maximum of 10 ma./cm.<sup>2</sup> when an anodic potential of 1.5 volts is impressed on a carbon electrode therein; heating the fluoride or mixture of fluorides to a temperature of about  $1000^\circ$  to  $1400^\circ$  F. in a noncontaminating atmosphere; establishing in the bath a fluoborate ion concentration not exceeding about 20 percent by weight; establishing a current density at the cathode not exceeding about 400 milliamperes per square centimeter; the current density at the cathode being selected with reference to the fluoborate concentration to fall within the operating limits defined by the area LMNO of FIG. 2; and the current density at the cathode further being selected with reference to the bath temperature to fall within the operating limits defined by the area WXYZ of FIG. 3.
2. The invention of claim 1 wherein the current density at the cathode is selected with reference to the fluoborate concentration to fall within the operating limits defined by the area LPQ of FIG. 2 and wherein the current density at the cathode is further selected with reference to the bath temperature to fall within the operating limits defined by the area UVW of FIG. 3.
3. The invention of claim 1 wherein said fused salt bath comprises a mixture of 40 to 60 mol percent potassium fluoride and 60 to 40 mol percent lithium fluoride.
4. The invention of claim 3 wherein the fluoborate ion concentration is established by bubbling boron trifluoride gas into the fluoride mixture.
5. The invention of claim 4 wherein the bath is purified prior to the establishment of the fluoborate concentration by subjecting the fluorides to a heat and vacuum treatment.
6. The invention of claim 5 wherein said fluorides are subjected to a temperature of from  $110^\circ$  to  $480^\circ$  C. at a

pressure of from  $10^{-2}$  to  $10^{-6}$  mm. Hg for up to 200 hours.

7. A boron coated product obtained by the method of claim 2, the boron coating having a hardness of approximately 3000 HV, an elastic modulus in flexure of  $60 \times 10^6$  to  $70 \times 10^6$  p.s.i. and being coherent and amorphous.

8. A process for producing substantially pure coherent boron on a cathode by electrodeposition from a fused salt bath consisting essentially of a mixture of 40 to 60 mol percent potassium fluoride and 60 to 40 mol percent lithium fluoride comprising the steps of: 10 heating the bath to a temperature of about 1000° to 1400° F. in a noncontaminating atmosphere; establishing in the bath a fluoborate concentration of approximately 1 to 20 percent by weight by adding 15 potassium fluoborate thereto; purifying the bath by nonanodically introducing therein fine chips of elemental boron until the electrolyte becomes passive thereto; establishing a current density at the cathode not exceeding about 400 milliamperes per square centimeter; 20 the current density at the cathode being selected with reference to the fluoborate concentration to fall

within the operating limits defined by the area LMNO of FIG. 2; and the current density at the cathode further being selected with reference to the bath temperature to fall within the operating limits defined by the area WXYZ of FIG. 3.

#### References Cited

##### UNITED STATES PATENTS

|           |         |                |       |        |
|-----------|---------|----------------|-------|--------|
| 1,795,512 | 3/1931  | Schmidt et al. | ----- | 204—39 |
| 1,845,978 | 2/1932  | Hosenfeld      | ----- | 204—39 |
| 2,918,417 | 12/1959 | Cooper et al.  | ----- | 204—60 |
| 2,984,605 | 5/1961  | Cooper         | ----- | 204—60 |
| 3,030,284 | 4/1962  | Stern          | ----- | 204—60 |

##### FOREIGN PATENTS

|         |        |               |       |        |
|---------|--------|---------------|-------|--------|
| 989,807 | 4/1965 | Great Britain | ----- | 204—39 |
|---------|--------|---------------|-------|--------|

JOHN H. MACK, Primary Examiner

D. R. VALENTINE, Assistant Examiner

U.S. Cl. X.R.

204—39

UNITED STATES PATENT OFFICE  
CERTIFICATE OF CORRECTION

Patent No. 3,843,497 Dated October 22, 1974

Inventor(s) SID RUSSELL ET AL

It is certified that error appears in the above-identified patent  
and that said Letters Patent are hereby corrected as shown below:

Column 1, line 45 "patten" should be --pattern--.

Column 2, line 3 "prefered" should be --preferred--.

line 11 "m./cm<sup>2</sup>" should be --ma/cm<sup>2</sup>--.

Column 3, line 53 "mv./min" should be --mV/min--.

Column 4, line 64 "follwed" should be --followed--.

line 71, "is", second occurrence, should  
be -- it --.

Signed and sealed this 24th day of December 1974.

(SEAL)

Attest:

McCoy M. Gibson Jr.  
Attesting Officer

C. Marshall Dann  
Commissioner of Patents